

## UNITED STATES PATENT OFFICE.

JOHN K. TULLIS, OF NEW YORK, N. Y.

## TANNING MATERIAL AND PROCESS OF PRODUCING SAME.

No Drawing.

Application filed March 17, 1922. Serial No. 544,667.

This invention relates to a tanning material or agent and a tanning process by which I am enabled to effect a satisfactory tanning of hides by a single-bath process. This 5 single-bath process, as herein described, may be followed, when desired, by a further final tanning operation in order to bring about certain results that may be desired in particular cases.

10 In practicing this invention I make use of various chrome compounds, together with certain sulfates or a mixture of sulfates. I have found chromic acid salts, such for example as the sodium bichromate or the bichromate of potassium, to be suitable, although chromic acid itself may be used. One or more of these chrome compounds are mixed with sulfates such as aluminum and magnesium for example, and I have 15 found that this mixture gives a good tanning extract that may be used in a single-bath for tanning purposes, thus eliminating the necessity of first treating the hides in a bath to produce an initial or preliminary 20 tanning and then subsequently treating them in a different bath to complete the tanning operation. In this way considerable labor is saved and the operation does not have to be watched as closely as is the 25 case with a two-bath process.

The following is given as a specific example illustrating the invention. It is not intended to restrict the invention to the particular details given in this example, as 30 variations of materials, proportions, etc., can be made without departing from the spirit or scope of the invention.

I may prepare an aqueous solution containing about two parts by weight of sodium 35 bichromate, five parts of magnesium sulfate and four parts of aluminum sulfate. The sodium bichromate may be substituted wholly or in part by bichromate of potassium. The hide, after the usual beam-house 40 preparation, is immersed in or wet with the liquid mixture of sulfates and bichromate above referred to for a sufficiently long time for the tanning to take place. The time required will depend largely upon the nature

and thickness of the hide to be tanned, and 50 the concentration of the solution, and in general will vary from about three to six days. At the end of this time the hide has become well tanned so that the leather can be used for a variety of purposes without 55 further tanning being necessary.

In case, however, it is desired to use the leather for sole leather or the like, I find it advisable to subject the same to an additional tanning operation. For this final 60 tanning operation I may use well known tanning extracts, such as waste sulfite liquor; or vegetable tanning materials, such as man-grove, oak, hemlock, quebracho, or chestnut, etc.; or sulfite liquor mixed with these 65 vegetable tanning materials; or formaldehyde sulfonic acid or other synthetic tanning agents. The one-bath tanning operation of my invention does not interfere with the final tanning above mentioned 70 when it is desired to use the latter for special purposes after the hide has been subjected to the tanning operation with the mixture of sulfates and the chrome compound.

## I claim:—

1. A composition to be used in a tanning process comprising, a bichromate, magnesium sulfate, and aluminum sulfate.
2. A composition to be used in a tanning process comprising sodium bichromate, magnesium sulfate, and aluminum sulfate.
3. A composition to be used in a tanning process comprising sodium bichromate, magnesium sulfate, and aluminum sulfate in the 85 proportions of about 2 to 5 to 4 by weight.
4. The step in the process of tanning hides which comprises treating a hide with a mixture of a chromic acid salt and magnesium and aluminum sulfates.
5. The step in the process of tanning hides which comprises treating a hide with an aqueous solution of a salt of chromic acid, magnesium sulfate and aluminum sulfate in substantially the proportions of 2 to 5 to 95 4 by weight.

In testimony whereof I affix my signature.  
JOHN K. TULLIS.